

## 1

2,744,063

## ELECTRODEPOSITION OF TIN-ANTIMONY-COPPER ALLOYS

Quentin O. Shockley, Indianapolis, Ind., assignor to General Motors Corporation, Detroit, Mich., a corporation of Delaware

No Drawing. Application December 11, 1951,  
Serial No. 261,153

8 Claims. (Cl. 204—44)

The present invention relates to a method and bath for alloy electroplating and is more particularly concerned with the electroplating of alloys containing tin, copper and antimony.

Alloys of tin, copper and antimony, and more particularly the tin base alloys containing copper and antimony, have long been accepted as satisfactory bearing materials. However, to prepare these alloys it has always been necessary to cast them from the molten state. In accordance with my invention such alloys are electrodeposited, thus accomplishing considerable simplification in manufacturing methods and procedure. A bearing metal layer, for example, can be plated on to a backing metal and the thickness of the metal layer closely controlled so as to dispense with subsequent machining operations to remove excess metal. Also, in many instances, a superior bearing surface can be obtained by electroplating than can be accomplished by means of the casting process.

It is an object of this invention to provide a new and useful method and bath for electroplating alloys of tin, copper and antimony. Other objects and advantages of my invention will be apparent in the following description of the preferred embodiments.

Briefly, my invention consists in plating tin-copper-antimony alloys by electrodeposition from an aqueous bath containing the fluoborate salts of these metals. Bath additives, such as betanaphthol and glue may be added to the bath to improve the quality of the plate. Variations in the composition of the alloy can be accomplished by variations in the current density and in the anode composition as well as by variations in the concentrations of the various metals in the bath.

One particularly important use of the process and fluoborate bath of this invention is for the plating of babbitts. Tin base, tin-copper-antimony alloys, such for example as SAE 10, 11 and 12, have been found to be especially satisfactory for certain types of bearing surfaces. I have found that such alloys can be electrodeposited to give a smooth, hard, dense plate from a bath containing the fluoborate salts of tin, copper and antimony within the following range of concentrations:

|          | Grams per liter |
|----------|-----------------|
| Tin      | from 60 to 80   |
| Copper   | from 1 to 5     |
| Antimony | from 1 to 5     |

It is generally advantageous to add to the bath from .25 to 2 grams per liter glue, and to maintain the bath saturated with betanaphthol. At room temperature this amounts to approximately 1 gram per liter of betanaph-

## 2

thol. The pH is maintained at between 0 and 1, and temperatures of from 70 to 100° F. may be used. The anode may either be pure tin or else an alloy of tin and copper, such as an alloy containing about 95% tin and about 5% copper. I have used the cathode current densities of from 10 to 60 amperes per square foot in conjunction with this bath, depending upon the exact alloy composition desired.

From a bath having the above range of metal concentrations and using current densities and anode materials within the range set forth, smooth, dense alloy platings containing from 79 to 97% tin, from 2 to 12% antimony and from 1 to 8% copper, may be plated. The particularly useful bearing alloys, such as SAE 10, 11 and 12, fall within this range.

The following specific examples of baths and of plating conditions from within the above range, together with the alloy compositions obtained therefrom, will serve for purposes of illustration:

### Example I

Anode: Sn—95%, Cu—5%

Cathode current density: 30 amperes per square foot

Bath:

|    |              |                 |     |
|----|--------------|-----------------|-----|
| 25 | Tin          | grams per liter | 75  |
|    | Copper       | do              | 1.0 |
|    | Antimony     | do              | 1.0 |
|    | Boric acid   | do              | 20  |
|    | Glue         | do              | 1.0 |
|    | Betanaphthol | do              | 1.0 |
|    | pH           |                 | 0.3 |
|    | Temperature  | ° F.            | 75  |

Agitation: Revolving anode

Deposit: Cu—1.5%, Sb—1.5%, Sn—balance.

### Example II

Anode: Sn—95%, Cu—5%

Cathode current density: 60 amperes per square foot

Bath:

|    |              |                 |     |
|----|--------------|-----------------|-----|
| 40 | Tin          | grams per liter | 62  |
|    | Copper       | do              | 3.5 |
|    | Antimony     | do              | 4.5 |
|    | Boric acid   | do              | 25  |
|    | Glue         | do              | 1.0 |
|    | Betanaphthol | do              | 1.0 |
|    | pH           |                 | 0.3 |
|    | Temperature  | ° F.            | 75  |

Agitation: Revolving anode

Deposit: Cu—2.6%, Sb—7.7%, Sn—balance.

### Example III

Anode: Sn—95%, Cu—5%

Cathode current density: 60 amperes per square foot

Bath:

|    |              |                 |     |
|----|--------------|-----------------|-----|
| 55 | Tin          | grams per liter | 65  |
|    | Copper       | do              | 3.0 |
|    | Antimony     | do              | 3.0 |
|    | Boric acid   | do              | 20  |
|    | Glue         | do              | 2.0 |
|    | Betanaphthol | do              | 1.0 |
|    | pH           |                 | 0.3 |
|    | Temperature  | ° F.            | 75  |

Agitation: Revolving anode

Deposit: Cu—6.3%, Sb—5.1%, Sn—balance.

**3**  
*Example IV*

Anode: 100% Sn  
Cathode current density: 60 amperes per square foot  
Bath:

|                        |                 |     |
|------------------------|-----------------|-----|
| Tin -----              | grams per liter | 75  |
| Copper -----           | do              | 1.5 |
| Antimony -----         | do              | 1.5 |
| Boric acid -----       | do              | 20  |
| Glue -----             | do              | 1.0 |
| Betanaphthol -----     | do              | 1.0 |
| pH -----               |                 | 0.3 |
| Temperature ----- ° F. |                 | 75  |

Agitation: Revolving anode

Deposit: Cu—8.9%, Sb—11.2%, Sn—balance.

*Example V*

Anode: 100% Sn  
Cathode current density: 30 amperes per square foot  
Bath:

|                        |                 |     |
|------------------------|-----------------|-----|
| Tin -----              | grams per liter | 75  |
| Copper -----           | do              | 1.5 |
| Antimony -----         | do              | 3.5 |
| Boric acid -----       | do              | 15  |
| Glue -----             | do              | .5  |
| Betanaphthol -----     | do              | 1   |
| pH -----               |                 | 0.3 |
| Temperature ----- ° F. |                 | 75  |

Agitation: Revolving anode

Deposit: Cu—1.0%, Sb—6.1%, Sn—balance.

For solution makeup and for concentration control I have found that a tin fluoborate concentrate containing approximately 300 grams per liter of stannous tin is satisfactory for addition of the tin constituent. For addition of the copper constituent a copper fluoborate concentrate containing approximately 180 grams per liter of copper can be used. The required antimony may be supplied in a number of ways. Antimony trioxide, antimony trifluoride, potassium antimony tartrate, and antimony fluoborate have all proved satisfactory. I have found that an antimony fluoborate solution containing approximately 35% antimony fluoborate, 9% fluoboric acid, and .3% hydrofluoric acid, to be the most convenient source of the antimony addition. In all cases, irrespective of the type of addition solution used, it has been found best to add the antimony compound as the last ingredient and after pH adjustment, since at this stage the antimony compound is most soluble and thus no difficulty is had from precipitants.

To adjust and maintain the pH, additions of a 42% commercial fluoboric acid solution can be made. I have found it preferable to add about from 10 to 40 grams per liter and preferably from 15 to 25 grams per liter of boric acid to the bath and then adjust and maintain the pH to that desired by additions of fluoboric acid.

The glue concentration is obtained by the addition of liquid glue obtained by dissolving bone glue pellets in a minimum amount of water. To maintain the solution saturated with betanaphthol, an excessive amount of this additive can be stirred into the solution and, after a period of agitation, the undissolved material filtered out.

While I prefer to use an anode consisting of either pure tin or else of an alloy of tin and copper, it is to be understood, of course, that an insoluble anode such as carbon

or platinum may be used. The chief advantage of a tin or of a tin-copper alloy anode is that it assists in maintaining the metal concentration of the solution. Anodes containing antimony have been found to be somewhat disadvantageous in that they sludge excessively.

It is generally preferable to agitate the bath solution during plating. This I accomplish by the use of a revolving anode; however, any suitable agitating means of course be used.

From the above listed examples it is apparent that differences in operating conditions and differences in bath concentrations result in very significant variations in the deposited alloy. It has been recognized, for example, that variations in anode composition and position have pronounced effect on the composition of the deposit. For example, using a bath having a composition of:

|                        |                                               |
|------------------------|-----------------------------------------------|
| Tin -----              | 75 grams per liter                            |
| Copper -----           | 1.5 grams per liter                           |
| Antimony -----         | 3.5 grams per liter                           |
| Glue -----             | 1 gram per liter                              |
| Betanaphthol -----     | Saturated solution (approx. 1 gram per liter) |
| pH -----               | .3                                            |
| Temperature ----- ° F. | 75° F.                                        |

The following deposits were obtained under the conditions specified:

1. Rotating (approx. 80 R. P. M.) internal anode (95% Sn and 5% Cu) 60 amperes per square foot cathode current density. Deposit analysis: 5.5% Sb, 2.8% Cu, 91.7% Sn.
2. Stationary external anode (95% Sn and 5% Cu) and rotating cathode (approx. 80 R. P. M.) 60 amperes per square foot cathode current density. Deposit analysis: 3.6% Sb, 2.3% Cu, 94.1% Sn.
3. Stationary external anode (pure Sn) and rotating cathode (approx. 80 R. P. M.) 60 amperes per square foot cathode current density. Deposit analysis: 1.2% Sb, 1.5% Cu, 97.7% Sn.

The choice of location of the anode, that is, the choice of whether it is to be internal or external, will of course depend upon the shape of the base metal being plated. Where, for example, the interior surface of a bearing shell is to be plated, an internal anode is used. When an external anode such as a cylinder is used, then agitation can be accomplished by the use of a revolving cathode, which is, of course, the article being plated.

It will be apparent that under closely controlled conditions, various useful tin base tin-copper-antimony alloys within a wide range can be plated with our bath and process.

While the process and bath of my invention can be used, as above, to electrodeposit Sn base alloys within the range of about 79 to 97% Sn, 2 to 12% Sb, and 1 to 8% Cu, it can also be used to plate other tin-copper-antimony alloys. A bath having metal ion concentrations with the range of from 50 to 180 g./l. tin, from .5 to 20 g./l. copper and from .5 to 20 g./l. antimony, and containing fluoboric acid and boric acid and preferably glue and betanaphthol within the ranges previously set forth, may be used. The current density can be from 10 to 60 amperes per square foot, the anode material being either pure tin, an alloy of tin and copper, or else an insoluble such as carbon or platinum. As in the case of the previously mentioned baths, the temperature may be from 70 to 100° F. I have obtained alloys containing from 1.5% to 99% tin, from .4% to 15.5% antimony and from .2% to 98% copper with my process, the exact percentage composition depending upon the various metal ion concentrations in the bath and also upon the condi-

tions used. The following table lists various plating baths and conditions along with the alloy deposited therefrom:

containing from 50 to 180 g./l. tin as tin fluoborate, from .5 to 20 g./l. antimony as antimony fluoborate, from .5

| Cathode Type | Anode    |              | Solution Concentration, g./l. |          |        | Current Density, Amps. per sq. ft. | Deposit           |                 |              |
|--------------|----------|--------------|-------------------------------|----------|--------|------------------------------------|-------------------|-----------------|--------------|
|              | Position | Composition  |                               | Antimony | Copper | Tin                                | Antimony, Percent | Copper, Percent | Tin, Percent |
|              |          | Tin, Percent | Copper, Percent               |          |        |                                    |                   |                 |              |
| Shell        | Internal | 100          |                               | 70       | 2      | 4                                  | 35                | 0.4             | 11.4         |
| Do.          | do       | 100          |                               | 80       | 2      | 10                                 | 35                | 0.4             | 15.2         |
| Do.          | do       | 100          |                               | 90       | 10     | 10                                 | 35                | 0.4             | 67.2         |
| Do.          | do       | 100          |                               | 125      | 10     | 10                                 | 35                | 0.7             | 60.5         |
| Do.          | do       | 100          |                               | 175      | 19     | 10                                 | 35                | 0.7             | 97.6         |
| Do.          | do       | 100          |                               | 75       | 0.5    | 0.5                                | 35                | 1.1             | 0.2          |
| Do.          | do       | 100          |                               | 75       | 1.5    | 1.5                                | 35                | 0.7             | 1.6          |
| Do.          | do       | 100          |                               | 75       | 3.5    | 3.5                                | 35                | 7.6             | 11.9         |
| Do.          | do       | 100          |                               | 75       | 0.5    | 0.5                                | 60                | 1.1             | 0.3          |
| Do.          | do       | 100          |                               | 75       | 1.5    | 1.5                                | 60                | 0.7             | 0.9          |
| Do.          | do       | 100          |                               | 75       | 3.5    | 3.5                                | 60                | 11.2            | 8.9          |
| Do.          | do       | 100          |                               | 75       | 10     | 10                                 | 60                | 15.5            | 29.4         |
| Do.          | do       | 100          |                               | 75       | 0.5    | 0.5                                | 10                | 0.4             | 2.0          |
| Do.          | do       | 95           | 5                             | 75       | 1.5    | 1.5                                | 10                | 0.6             | 4.0          |
| Do.          | do       | 95           | 5                             | 75       | 3.5    | 3.5                                | 10                | 14.6            | 23.1         |
| Do.          | do       | 95           | 5                             | 75       | 1.5    | 3.5                                | 35                | 15.3            | 1.3          |
| Plug         | External | 95           | 5                             | 75       | 1.5    | 3.5                                | 35                | 15.2            | 1.5          |
| Do.          | do       | 95           | 5                             | 75       | 1.0    | 1.0                                | 60                | 0.5             | 1.5          |
| Do.          | do       | 95           | 5                             | 75       | 2.5    | 2.5                                | 30                | 2.9             | 9.6          |
| Do.          | do       | 95           | 5                             | 75       | 2.5    | 2.5                                | 60                | 0.7             | 4.3          |
| Do.          | do       | 95           | 5                             | 75       | 2.5    | 4.5                                | 30                | 6.3             | 19.7         |

Satisfactory tin-antimony-copper alloys, and in particular those alloys containing a preponderance of tin, can be electrodeposited with the fluoborate bath and process of this invention. By the close control of the 30 bath composition, current density, circulation, anode material and the conditions enumerated, excellent deposits of several thousandths and even of several hundredths of an inch thick can be obtained with close control over the exact composition of the deposit. The process and bath of this invention make possible the electrodeposition of smooth dense deposits of varying thicknesses which adhere to metal bases such as steel and other ferrous metals, copper, copper lead alloys, silver, nickel and other metals and alloys.

Various changes and modifications of the embodiments of the invention described herein may be made by those skilled in the art without departing from the spirit and principles of the invention.

I claim:

1. The process of electroplating an alloy containing from about 2 to 12% antimony, from about 1 to 8% copper and the balance tin which consists in electrodepositing the alloy from an aqueous bath containing from 50 to 180 g./l. tin as tin fluoborate, from .5 to 20 g./l. antimony as antimony fluoborate, from .5 to 20 g./l. copper as copper fluoborate, from 10 to 40 g./l. boric acid, and sufficient fluoboric acid to maintain the pH of said bath at less than 1, the current density being from 10 to 60 amperes per square foot.

2. A process in accordance with claim 1 in which the anode material is selected from a group consisting of pure tin and the tin-copper alloys predominantly of tin.

3. A process in accordance with claim 1 in which the bath contains from .25 to 2 g./l. glue and about 1 g./l. 60 betanaphthol.

4. An aqueous bath for the electrodeposition of an alloy containing from about 2 to 12% antimony, from about 1 to 8% copper and the balance tin, said bath

to 20 g./l. copper as copper fluoborate, from .25 to 2 g./l. glue, from 10 to 40 g./l. boric acid, about 1 g./l. betanaphthol and sufficient fluoboric acid to maintain the pH of said bath below 1.

5. A process for electrodepositing a ternary alloy containing from about 2 to 12% antimony, from about 1 to 8% copper and the balance tin consisting of passing a current sufficient to yield a current density of from 10 to 60 amperes per square foot between a cathode and an anode and through a bath containing from about 60 to 80 g./l. tin as tin fluoborate, from about 1 to 5 g./l. antimony as antimony fluoborate, from about 1 to 5 g./l. copper as copper fluoborate, from about 15 to 25 g./l. boric acid, and sufficient fluoboric acid to maintain the pH of said bath at below 1.

6. A process in accordance with claim 5 in which the bath contains from .25 to 2 g./l. glue, and is saturated with betanaphthol.

7. A process in accordance with claim 5 in which the anode material is selected from a group consisting of pure tin and tin-copper alloys predominantly of tin.

8. An aqueous bath for the electrodeposition of an alloy containing from about 2 to 12% antimony, from about 1 to 8% copper and the balance tin, said bath containing from 50 to 180 g./l. tin as tin fluoborate, from .5 to 20 g./l. antimony as a compound selected from the group consisting of antimony fluoborate, antimony trioxide, antimony trifluoride and potassium antimony tartrate, from .5 to 20 g./l. copper as copper fluoborate, from 10 to 40 g./l. boric acid and sufficient fluoboric acid to maintain the pH of said bath below 1.

#### References Cited in the file of this patent

#### UNITED STATES PATENTS

- |           |               |                |
|-----------|---------------|----------------|
| 2,455,554 | Brown         | Dec. 7, 1948   |
| 2,458,827 | Booe          | Jan. 11, 1949  |
| 2,523,160 | Struyk et al. | Sept. 19, 1950 |